

T. B. MUNROE,  
REINFORCED FIBROUS BOARD AND PROCESS OF PRODUCING THE SAME.  
APPLICATION FILED APR. 3, 1919.

1,335,910.

Patented Apr. 6, 1920.



Witness  
*John Carter*

234

Inventor  
*T. B. Munroe*

Attorney

# UNITED STATES PATENT OFFICE.

TREADWAY B. MUNROE, OF FOREST GLEN, MARYLAND, ASSIGNOR TO B. G. DAHLBERG,  
OF ST. PAUL, MINNESOTA.

## REINFORCED FIBROUS BOARD AND PROCESS OF PRODUCING THE SAME.

1,335,910.

Specification of Letters Patent.

Patented Apr. 6, 1920.

Application filed April 3, 1919. Serial No. 287,139.

To all whom it may concern:

Be it known that I, TREADWAY B. MUNROE, a citizen of the United States, residing at Forest Glen, in the county of Montgomery and State of Maryland, have invented certain new and useful Improvements in Reinforced Fibrous Board and Processes of Producing the Same; and I do hereby declare the following to be a full, clear, and exact description of the invention, such as will enable others skilled in the art to which it appertains to make and use the same.

This invention relates to reinforced fiber board material and process of producing the same, and has for its object to provide an article which will be more efficient in use, and a method which will be more simple and easy to carry out than those which have been heretofore proposed.

With these and other objects in view the invention consists in the novel structure of the article and in the novel steps and combinations of steps constituting the process, all as will be more fully hereinafter disclosed and particularly pointed out in the claims.

Referring to the accompanying drawings, forming a part of this specification in which like numerals designate like parts in all the views—

Figure 1 is a diagrammatic sectional view of a portion of an apparatus suitable for carrying out the present process;

Fig. 2 is a plan view partially broken away of a portion of the material made in accordance with this invention;

Fig. 3 is a sectional view of the material shown in Fig. 2;

Fig. 4 is an enlarged diagrammatic view illustrating the disposition of the fibers during the process of making the articles; and—

Fig. 5 is a sectional view of a slightly modified form of interior construction of the article.

1 indicates any suitable tank or container adapted to hold water or other liquid carrying the cellulose pulp material out of which the article is made, 2 any suitable traveling belt adapted to exert a predetermined pressure upon the pulp material after it is formed into a board like mass, and 3 any suitable drum or roller provided with a foraminous surface such as 4, and adapted to coact with the belt 2 in compressing the fibers to a sheet of predetermined thick-

ness. 5 represents any reinforcing material such as wire cloth or other suitable fabric which is conveniently supported in the form of a roll 6, and fed down under roller 7 located in the tank 1, and led out between the roller 9 carrying the belt 2, and the upper surface of the drum 3 as illustrated.

The belt 2 also passes around the guiding roller 10 and together with the drum 3 is given motion in the direction of the arrows 11 and 12 respectively by any suitable means, such as the belt 8.

The cellulose fiber material, out of which the insulating board constituting this invention is made, differs essentially from the ordinary paper board material commonly met with in the market, in that it is composed of at least three or four different classes of fibers.

The one class consists of abnormally large fibers or slivers 13 frequently 1/8 inch wide and 1/2 inch long or longer. Mixed with these slivers are thread like fibers 14, which may be say from 1/32 inch to 1/64 inch in diameter and from 1/2 inch to 1 inch in length. Mixed with the thread like and sliver like fibers is a third class of hair like fibers 15, whose diameters are say 1/100 of an inch to say 1/200 of an inch, and anywhere from 1/2 inch to 1 inch or even two inches long.

Mixed with these three classes of fibers 13, 14 and 15 just mentioned, is a fourth class of fibers which is or may be identical with the ordinary comparatively short and very fine fibers used in paper making.

These several classes of fibers are mixed to a suitable consistency in water preferably in the proportions of from less than 1 to 5 parts of fiber to 99 or more to 95 parts of water, and are fed down into the tank 1 from the well 30 in which the water level is maintained high enough to provide a sufficient pressure to force the mixture up through the reinforcing material 5 which catches some of the fibers, while others which pass through the openings in the said material 5 continue up to the traveling belt 2 as indicated by the arrows 16 in Fig. 1.

This said head or pressure further forces the water through the interstices of the foraminous surface 4 of the roller or drum 3

in the direction indicated by the arrows 17 in Fig. 1, but the fibers which are carried by the said water are substantially all caught by and deposited on the said belt 2 and surface 4. The belt 2 and surface 4 being preferably made of wire cloth of say from 10 to 14 mesh, the fibers as they are impelled by the stream of water in the direction of the arrows 18, felt or mass themselves against the under surface of the belt 2, and also against the outer surface 4 of the drum 3. In addition to this more or less of the fibers collect in the restricted space 19 between the traveling wire cloths 2 and 4, and are there entangled and interwoven with the fibers composing the felted sheet-like masses that collect on the surfaces of said cloths 2 and 4, thus producing a reinforced board in which the fibers are thoroughly felted and interwoven throughout its entire thickness. As the said cloths 2 and 4 continue to move the entire mass is lightly compressed between the roller 9 and the drum 3 to expel some of the water, and the board emerges at the point 20 containing from only 50% to 75% of water.

By locating the foraminous reinforcing material 5, however, between the traveling cloths 2 and 4, as indicated, a large portion of said fibers are forced up through the meshes 22 of said foraminous material 5, see Fig. 4, and another portion 23 and 24 of said fibers is caught on each side of said material 5, all as will be clear from said figure. It results from this that a pronounced interlacing, or felting action takes place on the under side of the foraminous material 5, and a lesser interlacing, or felting action of the fibers takes place on the upper side of said material, with the result that the said foraminous material 5 is thoroughly felted into the mass or body portion of the final board 25 as is indicated in Figs. 2, 3 and 4. The said foraminous material 5 being thus firmly anchored on the interior of the fiber board 25, it adds very greatly to the strength of said board and in fact gives the said board in a sense some of the properties of reinforced glass in that the said board may receive blows and other injuries without being punctured or destroyed.

The proportions of fiber to water above given, *i. e.* from 1 or less to 5 parts of fiber to 99 or more to 95 parts of water are very important, for they provide a stock mixture in which each individual fiber is completely suspended, which suspension results in the great majority of the fibers traveling lengthwise, much after the manner of a stick floating in a swiftly moving stream. This said endwise travel of the fibers has been found to produce a greatly improved felting action, for the majority of the fibers strike the foraminous surfaces 2 and 4 at substantially right angles thereto, and before they have a

chance to be flattened down upon said surfaces other fibers are deposited beside them, whereupon the entire mass becomes more completely interwoven and entangled than has heretofore been the case.

Owing to the relatively high percentage of water used the velocity through the machine is quite high. For example, in an apparatus producing a board 4 feet wide by 1/2 inch thick at the rate of 10,000 linear feet per 24 hours, from 10 to 20 pounds of fiber and from 175 to 250 gallons of water pass through the machine every minute. This said high velocity further increases the intermingling and interweaving of the deposited fibers.

In this connection it might be pointed out that the felting action utilized by the present invention is sharply distinguished from the so called felting in paper making, wherein it is the constant endeavor to have the short, fine fibers there used lie flat against the foraminous belts or screens, with only sufficient actual felting to give coherence to the sheet. In the present case however, it is essential that the long thread like fibers, the hair like fibers and the coarse sliver like fibers be all intimately interwoven, and felted throughout the entire thickness of the board, the short, fine fibers being used merely as a filler, and to give the board a more finished surface.

The peculiar nature of the above mentioned classes of fibers 13, 14 and 15 lend themselves to the incorporation of the wire cloth 5 or other foraminous material, in that the different coarsenesses of these said fibers cause the board 25 to be unusually porous and this porosity greatly facilitates the felting action of the finer fibers between the coarser fibers so that the wires or threads constituting the foraminous material 5 find themselves filling the interstices between the fibers while the fibers themselves are so interwoven as to make a more or less homogeneous mass.

Stated in other language, as is well known, cellulose fiber material made after the usual fashion of felting it is liable to form into more or less pronounced layers and when the board is subjected to hard usage, it is liable to flake along the planes of these layers and thus to develop an undesirable weakness in use. But owing to the differences in coarseness of the various fibers, as well as to the large quantity of water used and its velocity through the apparatus, as above explained, this particular board not only has its layers much less pronounced than would otherwise be the case, but the strands of the wire cloth 5 serve to fill up to a greater or less degree the interstices between the individual fibers and thus bind the various layers together to a greater or less extent. This binding action is some-

what enhanced in the modified form of board illustrated in Fig. 5. In this figure the foraminous material 5 instead of being substantially in a single plane as indicated in Fig. 3, is zig-zagged or built into different planes so that a point such as 26 of said foraminous material will be located in one plane of the board 25 while another point 27 of said foraminous material will be located in an entirely different plane. The strands joining the point 26 and 27 will pass through a plurality of layers and thus will more or less firmly bind all the layers together. After the reinforcing fabric 5 has been thus incorporated into the pulp like mass, and after the desired pressure has been exerted upon said mass by means of the rollers or drums 3 and 9, the wet felted material may be passed to a suitable drying chamber or machine, dried out, cut into suitable lengths, or handled by other known methods as may be desired.

The material may be easily waterproofed or fireproofed to most any desired conditions of use, by introducing the waterproofing or fireproofing material in to the tank 1, or other suitable apparatus not shown and thoroughly mixing the same with the fibers or the finished sheet may be coated on the outside by any suitable means with the desired waterproofing or fireproofing material. For example, if it is desired to waterproof the board, a suitable proportion of ordinary rosin size, say 10% may be added to the stock in the well 30, or at other suitable place not shown and thoroughly mixed therewith. Aluminum sulfate may then be added to precipitate aluminum resinate and free rosin, which, due to the fact that each fiber is completely suspended as above pointed out, coats each individual fiber with a waterproofing compound, the material is then felted as above described, and issues from the machine containing from 50% to 85% of water.

It will of course be necessary to get rid of this surplus water before the board will be waterproofed and this may be done in any suitable manner, as for example, by heating. In this step, however, care must be taken to dry the board progressively from the interior outwardly, for if the outer portions are dried first they become waterproof, and it is then impossible to get the remaining water from the interior portions.

To this end I prefer to dry the boards in a continuous drier preferably steam heated, in which the atmosphere is kept moist, so that the interior portions of the board dry first. If this method of drying is continued until the board contains not more than say 5% of water, a product is obtained which is thoroughly waterproof, possesses a good surface and is of great structural strength. The surface obtained is espe-

cially adapted to receive coatings of plaster, asphalt, paint, etc., but if desired it may be especially treated as by sanding.

The temperature of the drier should preferably be maintained at say from 250° F. to 350° F. so as to dry the board in the least possible time, without charring it.

On the other hand, if a fireproof material is desired, the stock or the finished boards may be treated in any suitable manner to produce such a result. I prefer, however, in this case to treat the material with a substance which is substantially insoluble in water, but which under the influence of moderate temperature, say 150° C. to 500° C. will break down into its constituent parts, either solid, liquid or gaseous, one or more of which will not support combustion. Or, with a substance which, under the influence of heat, will give off an inert gas, incapable of supporting combustion. For example, fiber thoroughly impregnated with ferrous oxalate,  $FeC_2O_4 \cdot 2H_2O$  is found to be substantially fireproof. The said ferrous oxalate, when raised to a temperature of approximately 160° C. decomposes into two molecules of water, one molecule of carbon dioxide  $CO_2$ , one molecule of carbon monoxide  $CO$  and one atom of iron. Of these, only the carbon monoxide will support combustion, but this is overcome by the preponderance of other gases, liquids, and solids, produced which will not support combustion.

Further, if desired, instead of applying the fireproofing material directly to the fiber, it may be formed thereon by the reaction of two or more substances capable of producing it. For instance, instead of applying the ferrous oxalate directly, ferrous sulfate which is water soluble may be mixed with the fiber stock which is then treated with oxalic acid to form the insoluble ferrous oxalate.

It will of course be apparent that the board may be produced without either the waterproofing or fireproofing; it may be produced with the waterproofing alone or with the fireproofing alone; or it may be produced with both the waterproofing and fireproofing all according to the use which is to be made of it.

The board material 25 without the reinforcing material 5 is so porous that it often does not possess a specific gravity higher than say .4 and often its specific gravity is much lower and in fact not higher than say .2 so that it constitutes an excellent heat insulating material. On the other hand, if a greater density is desired the said material 25 may be filled in any suitable manner with a dope or binder.

Again, should different degrees of tenacity be desired in the finished product the woven material may be discontinuously fed into the felted mass during the course of manufac-

ture or the woven material 5 itself may be made of different strengths at different portions of its length.

It is obvious that those skilled in the art 5 may vary the details of construction as well as the procedure for producing the fiber board without departing from the spirit of the invention, and therefore, I do not wish to be limited to the above disclosure except 10 as may be required by the claims.

What I claim is:

1. The process of increasing the strength of fibrous board material which consists in felting the fibers against separated traveling surfaces; felting other fibers on a reinforcing material located between said traveling surfaces; and felting all of said fibers together with still other fibers to form a single adhering mass, substantially as described.

2. The process of making a reinforced board of fibrous material which consists in felting a layer of fibers on a traveling foraminous surface; felting a second layer of fibers on a second foraminous surface traveling in the same direction as said first surface; felting a third layer of fibers on a reinforcing fabric traveling in the same direction as said first and second named surfaces; and depositing other fibers in the spaces between said felted layers of fibers whereby all of said fibers are felted together into a single mass, substantially as described.

3. The process of making a reinforced board of fibrous material which consists in felting a layer of fibers on a traveling foraminous surface; felting a second layer of fibers on a second foraminous surface, traveling in the same direction as said first surface; felting a third layer of fibers on a reinforcing fabric traveling in the same direction as said first and second named surfaces; depositing other fibers in the spaces between said felted layers of fibers whereby all of said fibers are felted together into a single mass; compressing said mass lightly to remove a portion of the water contained therein; suitably removing substantially all of the remaining water therefrom; and cutting the same into suitable lengths, substantially as described.

4. As a new article of manufacture a

board made of fibers some of which are in the form of slivers, and having embedded in its main body portion a reinforcing foraminous material with a portion of the fibers on each side of said material interlaced with each other through its interstices, substantially as described.

5. As a new article of manufacture a 60 board composed of sliver like and finer fibers and having a specific gravity not higher than four tenths, said board also having embedded in its main body portion a reinforcing foraminous material with a portion of the fibers on each side thereof interlaced with each other through its interstices, substantially as described.

6. As a new article of manufacture a 70 board composed of coarse sliver like and finer fibers and having a specific gravity not higher than four tenths, said board also having embedded in its main body portion a reinforcing woven foraminous wire cloth 75 fabric with a portion of the fibers on each side of said fabric felted together through its openings, substantially as described.

7. As a new article of manufacture a 80 board composed of coarse sliver like and finer fibers and having a specific gravity not higher than four tenths, said board having incorporated therewith a water proofing material and also having embedded in its main body portion, a reinforcing woven foraminous wire cloth fabric with a portion of the 85 fibers on each side of said fabric felted together through its openings, substantially as described.

8. The process of making a porous fibrous board with a foraminous material embedded 90 in its body which consists in floating a mass of sliver like fibers mixed with other finer fibers in water on each side of said foraminous material while moving the latter; causing said water and a portion of said fibers to 95 pass in opposite directions through the openings of said material to interlace some of the fibers in said openings; and applying pressure to the mass of fibers on each side of said material to form the board, substantially as 100 described.

In testimony whereof I affix my signature.

TREADWAY B. MUNROE.